



US005506093A

**United States Patent** [19]**Kaplan et al.**[11] **Patent Number:** **5,506,093**[45] **Date of Patent:** **Apr. 9, 1996**[54] **IMAGING ELEMENT FOR REDUCTIVE  
LASER-IMAGING**[75] Inventors: **Mark S. Kaplan; Mitchell S. Burberry, both of Webster; Charles D. DeBoer, Rochester; Lee W. Tutt, Webster, all of N.Y.**[73] Assignee: **Eastman Kodak Company, Rochester, N.Y.**[21] Appl. No.: **380,479**[22] Filed: **Jan. 30, 1995****Related U.S. Application Data**

[63] Continuation-in-part of Ser. No. 205,531, Mar. 4, 1994.

[51] **Int. Cl.<sup>6</sup> ..... G03C 5/16**[52] **U.S. Cl. ..... 430/353; 430/332; 430/336;  
430/341; 430/936; 430/944**[58] **Field of Search** ..... 430/341, 944,  
430/336, 332, 936, 353[56] **References Cited**

## U.S. PATENT DOCUMENTS

|           |         |                              |
|-----------|---------|------------------------------|
| 3,628,953 | 12/1971 | Brinckman .                  |
| 4,247,625 | 1/1981  | Fletcher et al. .... 430/336 |
| 4,259,424 | 3/1981  | Endo et al. .... 430/619     |
| 4,410,623 | 10/1983 | DoMinh et al. .... 430/341   |
| 4,948,707 | 8/1990  | Johnson et al. .... 430/330  |

*Primary Examiner*—Thorl Chea  
*Attorney, Agent, or Firm*—Harold E. Cole

[57] **ABSTRACT**

This invention relates to an imaging element for reductive laser-imaging comprising a support having thereon an imaging layer comprising:

- a) a reducible Co(III) ammine complex,
- b) a source of phthalaldehyde, and
- c) a reducing agent,

the imaging layer having an infrared-absorbing material associated therewith in the amount of about 0.001 to about 0.5 g/m<sup>2</sup> of element.

**12 Claims, No Drawings**

# IMAGING ELEMENT FOR REDUCTIVE LASER-IMAGING

## CROSS-REFERENCE TO RELATED APPLICATIONS

This application is a continuation-in-part of U.S. Ser. No. 08/205,531, of Kaplan et al., filed Mar. 4, 1994.

This invention relates to the use of an imaging element for a reductive laser-imaging system which is useful for printing monochrome images developed by simple heating in the absence of chemical developing agents.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to the cyan, magenta or yellow signal. The process is then repeated for the other two colors. A color hard copy is thus obtained which corresponds to the original picture viewed on a screen. Further details of this process and an apparatus for carrying it out are contained in U.S. Pat. No. 4,621,271, the disclosure of which is hereby incorporated by reference.

Another way to thermally obtain a print using the electronic signals described above is to use a laser instead of a thermal printing head. In such a system, the donor sheet includes a material which strongly absorbs at the wavelength of the laser. When the donor is irradiated, this absorbing material converts light energy to thermal energy and transfers the heat to the dye in the immediate vicinity, thereby heating the dye to its vaporization temperature for transfer to the receiver. The absorbing material may be present in a layer beneath the dye and/or it may be admixed with the dye. The laser beam is modulated by electronic signals which are representative of the shape and color of the original image, so that each dye is heated to cause volatilization only in those areas in which its presence is required on the receiver to reconstruct the color of the original object. Further details of this process are found in GB 2,083,726A, the disclosure of which is hereby incorporated by reference.

U.S. Pat. No. 4,247,625 discloses an imaging element employing a reaction product of a cobalt complex and an aromatic dialdehyde which reacts with ammines generated in response to activating radiation. The activating radiation is used to excite a photo-activated photoreductant which, after activation, reduces cobaltic to cobaltous ammine complex salt. The photoreductant materials generally absorb in the blue and UV portions of the spectrum. The resulting films are therefore of low contrast in the blue and UV portion of the spectrum. In addition, the exposing device must emit in the blue and UV portions of the spectrum.

There is a problem with the above prior art in that there exists no heat-developable imaging element which a) can be exposed by a diode laser source, b) is of high resolution and

contrast, free from "flare," and c) which is of high contrast in the blue and ultraviolet (UV) regions of the spectrum.

It would be desirable to provide an imaging element that can be exposed by a diode laser source, that can be developed by thermal energy alone, that will provide images of high contrast in the blue and UV regions of the spectrum, and which provides images of high resolution free from flare.

These and other objects are achieved in accordance with this invention which relates to an imaging element for reductive laser-imaging comprising a support having thereon an imaging layer comprising:

- a) a reducible Co(III) aremine complex,
- b) a source of phthalaldehyde, and
- c) a reducing agent,

the imaging layer having an infrared-absorbing material associated therewith in the amount of about 0.001 to about 0.5 g/m<sup>2</sup> of element. In a preferred embodiment of the invention, a binder is also employed in the imaging layer.

Cobalt(III) ammine complexes useful in the invention generally have at least two ammonia ligands and include the following:



wherein X is a suitable anion and n is the number of atoms necessary to satisfy charge neutralization.

The above cobalt ammine complexes may be employed in amounts ranging from about 0.1 g/m<sup>2</sup> to about 5 g/m<sup>2</sup> of the imaging layer.

A source of phthalaldehyde includes phthalaldehyde:



as well as adducts of phthalaldehyde as disclosed in columns 3-9 of U.S. Pat. No. 4,410,623, the disclosure of which is hereby incorporated by reference.

A preferred class of phthalaldehyde adducts include the following:



wherein

$Z^1$  is the number of atoms necessary to complete two, or three carbocyclic or heterocyclic rings of from 9 to 13 nuclear atoms;

$Q$  is 0,



$>\text{NSO}_2\text{R}^2$ , or  $\text{S}$ ;

$Y$  is  $-\text{OH}$ ,  $-\text{OR}^5$ ,  $-\text{CHR}^3\text{R}^4$ ,



or  $-\text{NR}^6\text{R}^7$ ,

$\text{R}^1$  is



$\text{R}^2$  is alkyl or alkaryl of from 1 to 11 carbon atoms, for example, methyl, ethyl, propyl, isopropyl, p-methylphenylene, p-ethylphenylene and the like, the terms alkyl and alkaryl being understood to include those that are substituted in the alkyl portion, for example, p-(1-hydroxyethyl)phenylene;

$\text{R}^2$  further includes aryl or aralkyl of from 6 to 11 carbon atoms, for example, phenyl, naphthyl, benzyl, and the like, the term "aryl" being understood to include, in this context, substituted aryl, for example, aryl having halogen, nitro, alkyl, alkoxy,  $\alpha$ -hydroxyalkyl, dialkylamino and/or



substituents. (In some examples herein, the convention followed for the substituents on the carbo- or heterocyclic rings is that hydrogen substituents are not shown since they are obvious.)

$\text{R}^3$  and  $\text{R}^4$  are the same or different and are each hydrogen,  $-\text{SO}_3\text{CH}_3$ ,  $\text{NO}_2$ , or alkyl of from 1 to 5 carbon atoms, for example, methyl, ethyl, propyl, isopropyl and the like;

$\text{R}^5$  is alkyl of from 1 to 5 carbon atoms, for example, methyl, ethyl, propyl, isopropyl and the like; or is



and

$\text{R}^6$  and  $\text{R}^7$  are individually H or  $\text{SO}_2\text{R}^2$ , or together comprise the atoms necessary to complete a ring having the structure



5

10

15

20

25

30

35

40

45

50

55

60

65

$\text{X}$  is halogen, such as chlorine, bromine, iodine, and fluorine; and  
 $n$  is 1, 2, or 3.  
 Specific adducts of phthalaldehyde are:



Compound A



Compound B

The above phthalaldehyde or adducts thereof may be employed in amounts ranging from about 0.1 g/m<sup>2</sup> to about 10 g/m<sup>2</sup> of the imaging layer.

Examples of suitable reducing agents useful in the invention include the following:

dimethylhydantoin

3,4-dihydroxy-benzonitrile

1-naphthyl disulfide

thioctic acid

10-diazoanthrone

or any of the materials listed in Table II, columns 4-5 of U.S. Pat. No. 4,294,912, the disclosure of which is hereby incorporated by reference.

The above reducing agents may be employed in amounts ranging from about 0.1 g/m<sup>2</sup> to about 5 g/m<sup>2</sup> of the imaging layer.

Upon exposure of the imaging element to a laser beam, Co(III) is reduced to Co(II), and ammonia is produced during this reduction of the cobaltammine complex which then interacts with the phthalaldehyde to produce an intense black dye in the imaged areas. The thermal images obtained with such a medium are free of flare and exhibit high resolution and contrast.

A process of forming an image according to the invention comprises imagewise-heating, by means of a laser, an imaging element for reductive laser-imaging comprising a support having thereon an imaging layer comprising:

a) a reducible Co(III) ammine complex,

b) a source of phthalaldehyde, and

c) a reducing agent,

the imaging layer having an infrared-absorbing material associated therewith, and then thermally developing the element using heat. In a preferred embodiment of the invention, the heating step comprises heating with a hot

block or roller at a temperature of from about 90° C. to about 200° C. for a period of at least about 2 seconds.

The binder which may be employed in the imaging layer include materials such as cellulose acetate propionate, cellulose acetate butyrate, poly(vinyl butyral), nitrocellulose, poly(styrene-co-butyl acrylate), polycarbonates such as Bisphenol A polycarbonate, poly(styrene-co-vinylphenol) and polyesters. While any amount of binder may be employed in the layer which is effective for the intended purpose, good results have been obtained using amounts of about 0.1 to about 50 g/m<sup>2</sup>.

To obtain the laser-induced image of the invention, diode lasers are preferably employed since they offer substantial advantages in terms of small size, low cost, stability, reliability, ruggedness, and ease of modulation. In practice, before any laser can be used to heat an imaging element, the element must contain a laser light-absorbing material, such as carbon black, titanium dioxide or cyanine laser light-absorbing dyes as described in U.S. Pat. No. 4,973,572, or other materials as described in the following U.S. Pat. Nos.: 4,948,777, 4,950,640, 4,950,639, 4,948,776, 4,948,778, 4,942,141, 4,952,552, 5,036,040, and 4,912,083, the disclosures of which are hereby incorporated by reference.

Lasers which can be used in the invention are available commercially. There can be employed, for example, Laser Model SDL-2420-H2 from Spectra Diode Labs, or Laser Model SLD 304 V/W from Sony Corp.

Any material can be used as the support for the imaging element employed in the invention provided it is dimensionally stable and can withstand the heat of the laser. Such materials include polyesters such as poly(ethylene terephthalate); polyamides; polycarbonates; cellulose esters such as cellulose acetate; fluorine polymers such as poly(vinylidene fluoride) or poly(tetrafluoroethylene-co-hexafluoropropylene); polyethers such as polyoxymethylene; polyacetals; polyolefins such as polystyrene, polyethylene, polypropylene or methylpentene polymers; and polyimides such as polyimide-amides and polyether-imides. The support generally has a thickness of from about 5 to about 200 mm. It may also be coated with a subbing layer, if desired, such as those materials described in U.S. Pat. Nos. 4,695,288 or 4,737,486.

The following examples are provided to illustrate the invention.

#### Example 1 (IR-Absorbing Dye in Imaging Layer)

The following mixture was prepared and stirred until dissolved:

26.75 g cobalt hexaammine trifluoroacetate

83.25 g Compound A above

33.25 g dimethylhydantoin reducing agent

0.25 g IR-1 (see below)

144 g cellulose acetate propionate 482-0.5 (0.5 s viscosity)

enough acetone to make 1 liter total volume.



IR-absorbing dye IR-1

The solution was coated at 43 ml/m<sup>2</sup> on a 100 µm polyester support. After drying, the film was exposed to a diode laser beam on an apparatus described in U.S. Pat. No. 5,168,288. The exposure level was 200 mJ/cm<sup>2</sup> at 830 nm, with a 20 µm spot and a 10 µm line spacing. After exposure, the film was heated on a hot block held at 120° C. for the length of time required to develop the exposed image (about 6 s), but not long enough to develop any dye in the unexposed background (over 30 s). Microscopic inspection of the developed image revealed sharp, crisp edges, with no flare.

#### Example 2 (IR-Absorbing Dye in Adjacent Layer)

A mixture was prepared as in Example 1 except that it did not contain any IR dye. The solution was coated at 43 ml/m<sup>2</sup> on a 100 µm polyester support. After drying the film was overcoated with a solution of 5% Butvar B76® (poly(vinyl butyral) available from Monsanto Co.) and 0.1% IR-2 (below) in ethanol at 20 ml/m<sup>2</sup>. When dry, the film was exposed as in Example 1.

Microscopic inspection of the developed image again revealed sharp, crisp edges, with no flare. This example shows that the absorbing layer for the activating radiation does not have to be in the imaging layer but only has to be close enough to be able to heat the cobalt layer sufficiently to cause the reaction.



IR-absorbing dye IR-2

#### Example 3 (IR-Absorbing Metal in Adjacent Layer)

The mixture of Example 2 was coated at 43 ml/m<sup>2</sup> on 100 µm polyester support which had a layer of titanium 80 nm thick and a layer of TiO<sub>2</sub> over the titanium at a thickness sufficient to minimize reflection at 830 nm wavelength. After drying, the film was exposed as in Example 1.

Microscopic inspection of the developed image again revealed sharp, crisp edges, with no flare. This example shows that the absorbing layer for the activating radiation

does not have to be in the same layer as the cobalt or the reducing agent but only has to be close enough to be able to heat the cobalt layer sufficiently to cause the reaction. This experiment also shows that a metal layer also works equally well as an infrared-absorber.

The invention has been described in detail with particular reference to preferred embodiments thereof, but it will be understood that variations and modifications can be effected within the spirit and scope of the invention.

**What is claimed is:**

1. A process of forming an image comprising imagewise-exposing, by means of a laser, an imaging element for reductive laser-imaging comprising a support having thereon an imaging layer comprising:

- a) a reducible Co(III) ammine complex,
  - b) a source of phthalaldehyde, and
  - c) a reducing agent,

said imaging layer having an infrared-absorbing material associated therewith, and then thermally developing said element using heat.

  - 2. The process of claim 1 where the source of phthalaldehyde is phthalaldehyde.
  - 3. The process of claim 1 wherein a binder is present in said imaging layer.
  - 4. The process of claim 3 wherein said binder is cellulose acetate propionate.
  - 5. The process of claim 1 wherein said reducible Co(III) amine complex has at least two ammonia ligands.
  - 6. The process of claim 5 wherein said reducible Co(III) amine complex is

- 5      Co(III) (NH<sub>3</sub>)<sub>6</sub>(CF<sub>3</sub>-CO<sub>2</sub>)<sub>3</sub>  
       Co(III) (NH<sub>3</sub>)<sub>4</sub>(H<sub>2</sub>O)<sub>2</sub>(Cl<sup>-</sup>)<sub>3</sub>  
       [Co(III) (NH<sub>3</sub>)<sub>3</sub>(N<sub>3</sub>)<sub>3</sub>]  
       [Co(III) (NH<sub>3</sub>)<sub>5</sub>(C<sub>2</sub>O<sub>4</sub>)]<sup>1</sup>+X<sup>n</sup>  
       [Co(III) (NH<sub>3</sub>)<sub>4</sub>(C<sub>2</sub>O<sub>4</sub>)]<sup>1</sup>+X<sup>n</sup>  
       [Co(III) (NH<sub>3</sub>)<sub>2</sub>(C<sub>2</sub>O<sub>4</sub>)]<sup>1</sup>+X<sup>n</sup>  
       [Co(III) (NH<sub>3</sub>)<sub>3</sub>(H<sub>2</sub>O) (C<sub>2</sub>O<sub>4</sub>)]<sup>1</sup>+X<sup>n</sup>  
       [Co(III) (NH<sub>3</sub>)<sub>4</sub>(NO<sub>2</sub>) (N<sub>2</sub>H<sub>4</sub>)]<sup>2</sup>+X<sup>n</sup>  
 10     [Co(III) (NH<sub>3</sub>)<sub>3</sub>(H<sub>2</sub>O)<sub>3</sub>]<sup>3</sup>+X<sup>n</sup>  
       [Co(III) (NH<sub>3</sub>)<sub>3</sub> (N<sub>3</sub>)<sub>3</sub>]  
       [Co(III) (NH<sub>3</sub>)<sub>3</sub> (Cl<sub>3</sub>)]  
 15     wherein X is a suitable anion and n is the number of atoms  
       necessary to satisfy charge neutralization.  
 20     7. The process of claim 1 wherein said reducible Co(III)  
       ammine complex is cobalt hexaammine trifluoroacetate.  
       8. The process of claim 1 wherein said reducing agent is  
       dimethylhydantoin.  
 25     9. The process of claim 1 wherein said infrared-absorbing  
       material is a dye.  
       10. The process of claim 1 wherein said infrared-absorbing  
       material is located in a layer adjacent to said imaging  
       layer.  
 25     11. The process of claim 1 where said heating step is  
       performed at a temperature of from about 90° C. to about  
       200° C. for a period of at least about 2 seconds.  
       12. The process of claim 1 wherein said laser is an infrared  
       diode laser.

\* \* \* \*